

## UNITED STATES PATENT OFFICE

JOSEF NEUMANN, OF OFFENBACH-ON-THE-MAIN, GERMANY, ASSIGNOR TO GENERAL ANILINE WORKS, INC., OF NEW YORK, N. Y., A CORPORATION OF DELAWARE

## PRODUCTION OF COLORED RESISTING EFFECTS

No Drawing. Application filed June 24, 1930, Serial No. 463,584, and in Germany July 5, 1929.

The present invention relates to the production of colored resisting effects under ice colors by means of leuco ester salts of vat dyestuffs. According to the invention the goods are impregnated with any azo coupling component (such as an arylamide of 2-hydroxy-3-naphthoic acid, a naphthol or one of the derivatives of 1-hydroxy-naphthalene-4-carboxylic acid described in U. S. Patent 1,453,660), then the impregnated goods are imprinted with a printing paste containing an ester salt of a leuco-vat-dyestuff, an insoluble chromate which when acidified is capable of producing chromic acid and an alkali sulfite. Then the printed goods are dried and, without being previously steamed, developed with any diazo-compound, acidified and finished in the usual manner.

The favorable result attained was not to be foreseen because of the possibility of a mutual detrimental effect between the reducing alkali sulfite employed as a resist and the oxidizing chromate.

In order to further illustrate my invention the following examples are given, the parts being by weight and all temperatures in centigrade degrees, but it is however to be understood, that my invention is not limited to the particular products nor reacting conditions mentioned therein.—

## EXAMPLE 1

## Impregnating bath

35 15 grams of 2,3-hydroxy-naphthoyl-aniline  
22.5 cc. of caustic soda lye of 34° Bé.  
20 cc. of monopol-brilliant-oil are made up to

40 1 liter

## Resist of yellow

16 grams of the ester-salt of 3,4,8,9-dibenz-pyrene quinone, prepared according to U. S. Patent 1,564,584

|      |                                                     |    |
|------|-----------------------------------------------------|----|
| 10   | grams of glycerol                                   |    |
| 41.6 | grams of boiling water                              |    |
| 80   | grams of starch-tragacanth-thickening               |    |
| 10   | grams of mucilage of tragacanth                     | 50 |
| 14.4 | grams of lead chromate                              |    |
| 28   | grams of a solution of potassium sulfite of 45° Bé. |    |
| 200  | grams.                                              | 55 |

*Developing solution*

|     |                                                                     |    |
|-----|---------------------------------------------------------------------|----|
| 20  | grams of the diazonium-chloride of 4-amino-4'-methoxy-diphenylamine |    |
| 980 | grams of water                                                      | 60 |
| 1   | liter.                                                              |    |

The goods are impregnated, dried, printed with the resist, dried, developed and squeezed off. Then they are given a short passage c3 through air and then through a bath, heated to 80° C. of 30 cc. of hydrochloric acid of 20° Bé. per liter for a half a minute. Thereafter they are rinsed hot and cold and soaped at the boil for 3 minutes. 70

In this manner yellow effects on a blue ground are obtained.

## EXAMPLE 2

The goods are impregnated according to 75 Example 1 and printed with the following:

## Resist for blue

|      |                                                     |    |
|------|-----------------------------------------------------|----|
| 16   | grams of the ester-salt of hexa-bromo-indigo        | 80 |
| 10   | grams of glycerol                                   |    |
| 45.6 | grams of boiling water                              |    |
| 90   | grams of starch-tragacanth-thickening               |    |
| 10   | grams of mucilage of tragacanth                     | 85 |
| 14.4 | grams of lead chromate                              |    |
| 14   | grams of a solution of potassium sulfite of 45° Bé. |    |
| 200  | grams.                                              | 90 |

The goods are further treated according to Example 1.

Light blue effects on dark blue are thus obtained.

5

### EXAMPLE 3

The goods are treated according to Example 1, there being substituted for the resist the following resist for yellowish-green.

10

5 grams of the ester-salt of para-dichloro-dianilido-benzoquinone

11 grams of the ester-salt of the dyestuff prepared by oxydation of dibenzanthrone followed by ethylation

15

10 grams of glycerol

50.7 grams of boiling water

80 grams of starch-tragacanth-thickening

20

10 grams of mucilage of tragacanth

20

11.3 grams of barium chromate

22 grams of a solution of potassium sulfite of 45° Bé.

25

200 grams

The goods are dried, further developed with the diazo-solution according to Example 1 and finished in the same way. Yellow green effects on blue are thus obtained.

30

### EXAMPLE 4

The goods are impregnated according to Example 1, printed with the resist of Example 3, dried and then developed with a diazo-solution containing 10.5 grams of 5-nitro-2-toluidine per liter, to which sodium acetate has been added, and further treated as described in Example 1.

Yellow-green effects on a red ground are thus obtained.

### EXAMPLE 5

The goods are impregnated according to Example 1, printed with the resist of Example 3, dried and developed in the following:

#### Diazo-solution

20.6 grams of 1-amino-4-benzoylamino-2-methoxy-5-methyl-benzene are mixed with

6.9 grams of nitrite and 100 cc. of hot water; then the mass is cooled by adding

700 cc. of cold water,

23.6 cc. of hydrochloric acid of 20° Bé. are introduced and after some time

8.2 grams of sodium bicarbonate, dissolved in

60 cc. of water, and

21.8 grams of magnesium sulphate, dissolved in

60 cc. of water, are added and the whole is made up to

65 1 liter.

By working according to Example 1 yellow-green effects on a violet ground are obtained.

### EXAMPLE 6

70

#### Impregnating bath

22.5 grams of  $\beta$ -naphthol,

25.5 grams of caustic soda solution of 34° Bé.

20 grams of Turkey red oil, made up to 75 1 liter.

The goods are impregnated with this impregnating bath, dried and printed with the resist of Example 1. After drying, the goods are developed in a diazo-solution containing 21.5 grams of para-nitraniline per liter, to which sodium acetate is added, and finished in the same way.

In this manner yellow effects on a red ground are obtained.

### EXAMPLE 7

90

The goods are impregnated with the following

#### Impregnating bath

15 grams of 4-hydroxy-naphthalene-1-phenylketone

10 grams of caustic soda solution of 34° Bé.

20 grams of Turkey red oil, are made up to

1 liter;

they are then dried and printed with the resist of Example 2, dried and developed in a diazo-solution containing 8 grams of ortho-phenetidine per liter, to which chalk has been added, and finished as described above.

Blue effects on red are thus obtained.

### EXAMPLE 8

105

#### Impregnating bath

15 grams of 2',3'-hydroxy-naphthoyl-5-chloro-2-toluidine

30 grams of caustic soda solution of 34° Bé.

20 grams of Turkey red oil, are made up to

1 liter.

The goods are impregnated with this impregnating bath, dried and printed with the following

#### Resist for blue

16 grams of the ester salt of tetra-bromodigo,

10 grams of glycerol

32.7 grams of boiling water

70 grams of starch-tragacanth-thickening

11.3 grams of barium chromate

60 grams of a solution of potassium sulfite of 45° Bé.

200 grams.

After drying, they are developed in a diazo-

130

solution containing 19 grams of 5-chloro-2-toluidine hydrochloride per liter, to which sodium acetate has been added, acidified and finished in the same way.

5 Blue effects on a red ground are thus obtained.

I claim:—

1. Process which comprises impregnating textile goods with an azo coupling component, 10 imprinting the impregnated goods with a printing paste containing an ester salt of a leuco-vat-dyestuff, an insoluble chromate which when acidified is capable of producing chromic acid and an alkali sulfite, drying the 15 printed goods, developing them with any diazo-compound, acidifying and finishing them in the usual manner.

2. The process which comprises, impregnating textile goods with 2,3-hydroxy-naphthoyl aniline, imprinting the impregnated goods with a printing paste containing the ester salt of leuco 3,4,8,9-dibenzopyrenequinone, lead chromate and potassium sulfite, drying the printed goods, developing them 25 with the diazo compound of 4-amino-4'-methoxy-diphenylamine, acidifying and finishing them in the usual manner.

3. The process which comprises impregnating textile goods with 2,3-hydroxy-naphthoyl aniline, imprinting the impregnated goods with a printing paste containing the ester salt of leuco-hexabromindigo, lead chromate and potassium sulfite, drying the printed goods, developing them with the diazo compound of 35 4-amino-4'-methoxy-diphenylamine, acidifying and finishing them in the usual manner.

4. The process which comprises impregnating textile goods with 2,3-hydroxy-naphthoyl aniline, imprinting the impregnated goods 40 with a printing paste containing an ester salt of leuco-para-dichloro-dianilide-benzoquinone and the ester salt of the leuco vat dye-stuff prepared by oxidation of dibenzanthrone followed by ethylation, barium chromate and 45 potassium sulfite, drying the printed goods, developing them with the diazo compound of 4-amino-4'-methoxy-diphenylamine, acidifying and finishing them in the usual manner.

50 In testimony whereof, I affix my signature.

JOSEF NEUMANN.